

# UNITED STATES PATENT OFFICE.

WALTER OSTWALD, OF GROSSEBOHLEN, GERMANY, ASSIGNEE, BY MESNE ASSIGNMENTS, TO THE CHEMICAL FOUNDATION, INC., A CORPORATION OF DELAWARE.

METHOD OF OBTAINING BY-PRODUCTS, PARTICULARLY NITROGEN COMPOUNDS, FROM BLAST-FURNACES.

1,344,770.

Specification of Letters Patent. Patented June 29, 1920.

No Drawing. Application filed October 10, 1918. Serial No. 124,855. Renewed November 25, 1919. Serial No. 340,461.

To all whom it may concern:

Be it known that I, WALTER OSTWALD, a citizen of the German Empire, and residing at Haus Dowa, Grossbothen, Saxony, Germany, have invented a new and useful Improved Method of Obtaining By-Products, Particularly Nitrogen Compounds, from Blast-Furnaces.

A primary object of my invention is to obtain by-products, particularly nitrogen compounds, from blast furnaces.

The formation of nitrogen compounds in blast furnaces, particularly the formation of ammonia and ammonium chlorid, is connected with difficulties owing to there being no water vapor present in those zones of the furnace in which the formation of ammonia or ammonium chlorid can take place, for as the charge slowly sinks it is heated to a higher temperature than that required for expelling the moisture in it, and any water vapors which are produced are driven off with the other smelter gases before the charge has reached the temperature zone, in which the formation of ammonia or ammonium chlorid takes place. The gases flowing in the opposite direction *i. e.* from the bottom to the top of the furnace, contain no water vapor, because the blast is dried beforehand as much as possible, and any residual traces are decomposed at the very much higher temperatures in the lower parts of the furnace.

According to my invention nitrogen compounds are produced by introducing or generating water or steam in and introducing chlorids into that zone which has a temperature of 500° to 900° C., a temperature at which ammonia and ammonium chlorid can be formed. The most simple mode of procedure would be to introduce steam through the side wall of the furnace. In order to distribute the steam more evenly, however, I prefer to introduce the water necessary for the formation of ammonia or ammonium chlorid in the state of water contained in a hydrate. Further, the production of nitrogen compounds according to the present invention may be effected by adding salts which forms hydrates, particularly those which are rich in hydration water. The salts adapted for use in the process part with their hydrate water only at high tem-

peratures, some of them only at temperatures up to 600°. At this temperature, however, the formation of ammonia and ammonium chlorid has already commenced. By introducing water in the form of hydrate water into these highly heated zones it is possible, without disturbing the smelting process, to prevent or limit both the combustion of the bound nitrogen into free nitrogen, as well as the formation of cyanid, and instead thereof, to promote the formation of ammonia or ammonium chlorid according to the nature of the added hydrated salts. Chlorids may be used as such salts which form hydrates, in which case, the formation of ammonium chlorid is promoted. The chlorid ion constitutes an extremely effective protection against the combustion of ammonia into free nitrogen, which explains the high yield obtained. Obtaining nitrogen in the form of ammonium chlorid has the advantage that the separation, collection and refining of this nitrogenous compound is comparatively simple, and, in addition, the use and cost of sulfuric acid, which cannot be avoided when ammonium sulfate is produced in the usual manner, are obviated.

A further advantage obtained by using chlorids is that it is possible to obtain the ammonium chlorid in the form of an aqueous solution in a particularly simple manner by simply washing the gases. As blast-furnace gases are generally purified in any case by a wet process, the ammonium chlorid is found in the scrubbing water, so that no particular apparatus is required for its collection. Of the chlorids, calcium chlorid can be used with the great advantage that the lime is left behind in an extremely finely divided state after the splitting off of its hydrate water and its chlorid ion, so that the amount of lime normally added to the charge can be diminished.

A particularly fine and uniform distribution of the chlorin is obtained by quenching the coke with a salt solution. The hot coke eagerly absorbs the solution up to 25% of its weight, evaporates the water to a greater or less extent and after complete cooling still retains 8% water, a still larger percentage of the dissolved salt, however, remains in the coke. When a solution of

calcium chlorid is used the amount of lime contained in a finely divided form in the coke can be taken into proper consideration in the calculation of the mixture of ores and fluxes.

I claim:

1. In the manufacture of metals from a mixture of ores, fuel and fluxes in blast furnaces, the herein described method of obtaining as a by-product the nitrogen contained in the mixture, which consists in adding to the mixture a suitable quantity of a hydrated chlorid, whereby the water of hydration is liberated and converted into steam which acts on the mixture in the temperature zone in which ammonia is formed, whereby all the nitrogen of the fuel is converted into ammonium chlorid, and in separating the ammonium chlorid from the blast furnace gases, substantially as described.
2. In the manufacture of metals from a mixture of ores, fuel and fluxes in blast furnaces, the herein described method of obtaining as a by-product the nitrogen contained in the mixture which consists in adding to the mixture a suitable quantity of a chlorid, in causing steam to act on the mixture in the temperature zone in which ammonia is formed, whereby all the nitrogen of the fuel is converted into ammonium chlorid, and in separating the ammonium chlorid from the blast-furnace gases, substantially as described.

3. In the manufacture of metals from a mixture of ores, fuel and fluxes in blast furnaces, the herein described method of obtaining as a by-product the nitrogen contained in the mixture, which consists in adding to the mixture a suitable quantity of hydrated calcium chlorid, in liberating the water of hydration and in forming ammonia at a temperature of from 500° C. to 900° C., whereby all the nitrogen of the fuel is converted into ammonium chlorid, and in scrubbing the ammonium chlorid out of the blast-furnace gases, substantially as described.

4. In the manufacture of metals from a mixture of ores, coke and fluxes in blast furnaces, the herein described method of obtaining as a by-product the nitrogen contained in the mixture, which consists in quenching the coke of the mixture with a solution of calcium chlorid, in the liberation of water and in the formation of ammonia at a temperature of from 500° to 900° C., whereby all the nitrogen of the fuel is converted into ammonium chlorid, and in washing the ammonium chlorid out of the blast furnace gases, substantially as described.

Having thus described my invention, I have hereunto set my signature in the presence of two subscribing witnesses.

WALTER OSTWALD.

Witnesses:

RUDOLPH FRICKE,  
R. H. SEAGLE.